

Nov. 28, 1944.

O. SASLAW

**2,363,555**

## METHOD OF PRODUCING SELENIUM RECTIFIERS

Filed Aug. 21, 1943



OTTO INVENTOR.  
SASLAW

OTTO SASLAW

BY *George S. Joyde*  
ATTORNEY

## UNITED STATES PATENT OFFICE

2,363,555

METHOD OF PRODUCING SELENIUM  
RECTIFIERS

Otto Saslaw, Lyndhurst, N. J., assignor to Federal Telephone and Radio Corporation, New York, N. Y., a corporation of Delaware

Application August 21, 1943, Serial No. 499,526

4 Claims. (Cl. 175—366)

This invention relates to a method of making selenium rectifiers.

A selenium rectifier is generally made by uniting a layer of selenium with a metallic base plate, converting the selenium layer to the crystalline form by heat treatment, forming on the selenium a blocking layer which is responsible for the rectifying action, applying a counter-electrode and finally electro-forming. The blocking layer may be formed by depositing on the selenium layer in the presence of moisture a thin film of selenium dioxide, for example by vaporizing the dioxide and allowing it to condense on the selenium surface.

An important object of the invention is to improve a blocking layer of this type, and more specifically to decrease the reverse current characteristic of the rectifier without materially affecting its forward conductivity. It has been found that this can be done by depositing the selenium dioxide in an atmosphere of carbon dioxide and moisture on the selenium surface, prior to the application of the counter-electrode. The gas, vapor and selenium dioxide appear to cooperate to give an enhanced blocking effect. It has also been found that the blocking layer can be further improved if the electro-formation is carried out in the presence of CO<sub>2</sub> and moisture.

Other objects and advantages will appear from the following detailed description and the attached drawing in which:

Fig. 1 is a diagram illustrating a process embodying a specific form of the invention, and

Fig. 2 is a fragmentary diagram illustrating a process for the electro-forming of a selenium rectifier.

According to a specific embodiment of the invention, the process may be conveniently carried out by allowing carbon dioxide gas which has bubbled through hot water to contact the selenium surface and at the same time condensing on said surface fumes of selenium dioxide which has been heated to or above its evaporating temperature.

Referring to Fig. 1, which illustrates this embodiment, 1 represents a tank of compressed CO<sub>2</sub> gas which discharges through a pipe 2 into the lower part of a water tank 3 suitably heated as by steam coils 4 and having a gas outlet pipe 5 connected to the tank above the surface of the water and discharging into a hood 6. An assembly of rectifiers 7 to be fumed is suspended in hood 6 through an opening in the hood, as by an arm 8 attached to a handle 9 by which said assembly can be moved into or out of the hood.

enclosure. An electric furnace 10 for heating a crucible 11 containing selenium dioxide is located in the lower part of hood 6 in position for effective fuming of the lower surfaces of disks 7.

When the apparatus is in operation, the valve 12 of the tank 1 is opened to allow CO<sub>2</sub> gas to flow into the pipe 2, thence into the bottom of the water tank 3 which is conveniently kept at a temperature of 80-95° C., from which the gas emerges at the top carrying moisture, passing through the overhead pipe 5 into the hood 6 where the wet gas envelops the assembly of rectifiers arranged with their selenium surfaces exposed. At the same time, or shortly prior or subsequent thereto, the crucible 11 containing the selenium dioxide is heated to a temperature of approximately 400-500° C. to volatilize the oxide and cause it to be deposited on the free selenium surfaces.

After the selenium elements have taken up the required amounts of selenium dioxide, moisture and CO<sub>2</sub>, they are removed from hood 6 and each is provided with a metallic counter-electrode, as by spraying. It is desirable that this be done promptly inasmuch as it has been found that better rectifiers are produced when the counter-electrode is applied soon after deposition of the materials than when a long period of time is allowed to intervene. The delay should not exceed 30 seconds, and preferably is not more than 5 seconds.

At this stage the rectifiers are electro-formed by applying a rectified alternating current voltage for several hours in the direction of reverse current flow. An arrangement for this purpose is diagrammatically indicated in Fig. 2, in which the negative terminal of the source is connected to the metallic base plate 13 of the rectifier and the positive terminal is connected to the counter-electrode 14. The disks 7 during this operation are enclosed in a chamber 16 containing CO<sub>2</sub> and moisture, which may be introduced from tank 3 through pipe 17, the arrangement being such that the electro-forming step is carried out in an atmosphere of CO<sub>2</sub> and moisture.

The proper proportions of carbon dioxide and moisture will be obtained if the carbon dioxide is used at a pressure of from 1 to 20 pounds per square inch gauge pressure, and preferably approximately 5 pounds. The room humidity should be above 50%.

Although the process has been described with particular reference to a preferred embodiment involving the deposition of the selenium dioxide film on the selenium layer by means of vapo-

rization and condensation of the oxide on said selenium layer, the invention is not limited to this method of depositing the oxide, and any other convenient method may be used for this purpose. The method of introducing the moisture, while especially advantageous, is likewise disclosed by way of illustration rather than limitation.

What is claimed is:

1. In the manufacture of a selenium rectifier, the method of forming a blocking layer which comprises depositing a thin film of selenium dioxide on the selenium layer of a unit comprising a layer of selenium joined to a base plate, subjecting said selenium layer to an atmosphere of carbon dioxide and moisture and applying a counter-electrode to said selenium layer.

2. The method as set forth in claim 1 in which the selenium dioxide film is deposited on said

selenium layer in the presence of the carbon dioxide and moisture.

3. In the manufacture of a selenium rectifier, the method which comprises vaporizing selenium dioxide, causing said vapors to condense on a selenium layer supported on a base plate, in an atmosphere of carbon dioxide and moisture and immediately applying a counter-electrode to said selenium layer.

4. In the manufacture of a selenium rectifier, the method which comprises vaporizing selenium dioxide, causing said vapors to condense on a selenium layer supported on a base plate, in an atmosphere of carbon dioxide and moisture, applying a counter-electrode to said selenium layer and finally electro-forming said rectifier in an atmosphere of carbon dioxide and moisture.

OTTO SASLAW.